

# UNITED STATES PATENT OFFICE.

MARK A. ATUESTA, OF SCHENECTADY, NEW YORK, ASSIGNOR TO GENERAL ELECTRIC COMPANY, A CORPORATION OF NEW YORK.

## BLACK FINISH

1,157,283.

Specification of Letters Patent.

Patented Oct. 19, 1915.

No Drawing.

Application filed June 9, 1915. Serial No. 33,202.

To all whom it may concern:

Be it known that I, MARK A. ATUESTA, a citizen of the United States, residing at Schenectady, in the county of Schenectady, 5 State of New York, have invented certain new and useful Improvements in Black Finish, of which the following is a specification.

My invention relates to black finish for articles of cast and wrought iron, steel and 10 ferrous metal generally, my aim being to obtain a durable, uniform finish of good appearance that can be easily and expeditiously produced at a comparatively low cost.

Other advantages of my finish include 15 protection of the metal against rust and corrosion; absence of any heavy coating liable to flake off, or to mar the sharpness of angles or impair the meshing of threads; and certainty and uniformity of results.

How these and other advantages can be secured will be apparent from the following 20 description of the best way of producing my finish at present known to me; but while the invention extends even to the specific 25 features and details of the procedure herein-after described, it is not confined thereto,—its real scope being indicated in my claims.

After cleaning the articles or "material" 30 to be blacked, either by pickling or by shot or sand blasting, I give them a thin coating of zinc. This I prefer to do by a sherardizing process carried out in such a way that the coating shall not exceed .0015" in thickness, though material whose intended use 35 will expose it to severe corrosive influences may be more heavily coated. The sherardizing coat may be made thus light (as compared with that usually given when articles

40 are not to be otherwise coated) by shortening the time of treatment, lowering the treating temperature, or diminishing the amount of zinc dust used. The sherardized material is placed in hot charred bone dust 45 or its equivalent to which liquid coal tar has been added in the proportion of one quart of tar to fifteen quarts of bone dust. One quart of the bone dust thus prepared with tar for each eight pounds of sherardized 50 material to be treated represents good practice. The material is treated with the bone dust by heating it in a sherardizing drum to about 360° C., this temperature being maintained for about an hour and a half. Pref-

erably the temperature should not reach the 55 melting point of zinc (419° C.) or greatly exceed 375° C., in order to avoid risk of injury to the sherardizing coat. After removal from the drum and shaking off of the surplus dust, the material is placed in an 60 oven at a temperature of about 500° C., baked for about five minutes, and then quenched in boiled linseed oil. Thereafter the material may be "dried" or freed of adherent oil either by tumbling in it sawdust 65 or by means of a centrifugal oil separator. Apparently the bone dust (which is a phosphorus containing carbonaceous residue, consisting principally of calcium phosphate and free carbon) gives "body", the tar improves 70 the color of the coat, as well as its coherent and adherent properties, and the oil quenching makes it adhere more firmly; but there may be other equally important effects due 75 to the various substances.

It would appear that some reaction takes 80 place between the sherardizing coat (consisting principally of zinc) and the carbonaceous material employed in the foregoing procedure, so that the results as regards 85 quality and adhesion of the black coat are improved by the sherardizing. Nevertheless, the black finish can be applied to unsherdized material, and it offers such resistance to rust and corrosion as to render it 90 a sufficient protection in some cases. In such cases the above considerations as to injury of the zinc coat in the bone dust heat do not apply; but it is still best to observe about the same limit of temperature in order to 95 secure a black coating rather than a cementation with carbon, and, in the case of steel, to avoid scaling.

In order that the best results may be secured in the practice of my invention, I 95 will now describe briefly the method of sherardizing that I have found most suitable. For this operation I employ zinc dust in which the percentage of metallic zinc is 80 to 92%. Ordinary zinc dust of commerce is 100 usually too low in metallic zinc, so that I prefer to use zinc powder (which is artificially produced "atomized" metallic zinc) and to oxidize it to the extent indicated by a preliminary heating in a sherardizing drum. Save for zinc oxid, this powder should be as pure as possible,—and, especially, free from lead,—although very small quantities of 105

silica or iron oxid do not appear to be deleterious. I prefer to heat the material in this zinc powder in a lagged drum or furnace with suitable electrical heating units 5 or coils in its walls. The heating temperature should not vary much beyond the range of 350° C. to 375° C., and the charge should be brought up to this temperature as quickly as possible and kept there for about three 10 hours,—more or less,—according to the thickness of the coating desired, the size of the articles, etc. After each run the zinc metal content of the powder should be restored to its initial proportion by admixture 15 of fresh unoxidized powder (to make up for the oxidation during that run) before being used again. A close observance of these directions insures a smooth, even, uniform coat free from lumps, and allows its thickness 20 to be so accurately controlled by proper timing that bolts and nuts whose threads have been undercut sufficiently will fit exactly without reapplication of taps or dies;—and this likewise, after the black 25 finish has been given the articles.

What I claim as new and desire to secure by Letters Patent of the United States, is:—

1. The method of producing a rust-proof black finish on ferrous articles which consists in coating them with zinc, heating them 30 in charred bone dust mixed with carbona-

ceous binder, and subsequently quenching them in carbonaceous liquid.

2. The method of producing a rust-proof black finish on ferrous articles which consists in coating them with zinc, heating them in finely divided phosphorus-containing carbonaceous material mixed with black carbonaceous binder, and subsequently quenching them in oil. 35

3. The method of producing a rust-resisting black finish on ferrous articles which consists in heating them in charred bone-dust mixed with carbonaceous binder and subsequently quenching them in carbonaceous liquid. 40

4. The method of producing a rust-proof black finish on ferrous articles which consists in sherardizing them, heating them in charred bone dust mixed with tarry binder 50 at a temperature below the fusion point of the sherardizing coat, and subsequently quenching them in oil.

5. The method of producing a black finish on ferrous articles which consists in heating such articles in charred bone dust mixed with liquid coal tar and subsequently quenching them in boiled linseed oil. 55

In witness whereof, I have hereunto set my hand this 8th day of June, 1915.

MARK A. ATUESTA.